

F. A. FAHRENWALD.

COMPOSITION OF MATTER FOR PLATINUM SUBSTITUTE IN ELECTRICAL TERMINALS AND OTHER USES.

APPLICATION FILED FEB. 18, 1918.

1,339,505.

Patented May 11, 1920.



Inventor  
Frank A. Fahrenwald  
Attys  
Hull, Smith, Brock & West

# UNITED STATES PATENT OFFICE.

FRANK A. FAHRENWALD, OF CLEVELAND, OHIO, ASSIGNOR TO THE RHOTANIUM COMPANY, OF CLEVELAND, OHIO, A CORPORATION OF OHIO.

## COMPOSITION OF MATTER FOR PLATINUM SUBSTITUTE IN ELECTRICAL TERMINALS AND OTHER USES.

1,339,505.

Specification of Letters Patent. Patented May 11, 1920.

Original applications No. 108,991, filed July 13, 1916, and No. 129,911, filed November 6, 1916. Divided and this application filed February 18, 1918. Serial No. 217,835.

*To all whom it may concern:*

Be it known that I, FRANK A. FAHRENWALD, a citizen of the United States, residing at Cleveland, in the county of Cuyahoga and State of Ohio, have invented a certain new and useful Improvement in Composition of Matter for Platinum Substitute in Electrical Terminals and other Uses, of which the following is a full, clear, and exact description, reference being had to the accompanying drawings.

This invention relates to an improvement in alloys and has for its object to provide a composition of metal which may be employed in many cases as a substitute for metallic platinum and expensive platinum alloys in various types of electrical construction, as spark devices, resistance elements, thermo couple elements, etc., and in articles of jewelry, chemical containers, and the like, as well as in dentistry, philosophical instruments and surgery. The qualities of platinum which render it of such great use in these fields have been its hardness (especially when alloyed with iridium), its high melting point (which is also heightened by alloying with iridium or the like), and its resistance to oxidation and chemical action, which prevents it from erosion by electrical influences or from corrosion by acids or oxidizing influences.

The objects of my invention are the provision of an alloy material which shall be substantially equal to platinum in respect of hardness, melting point, and electrical and chemical resistivity so as to be usable for spark points, electrical terminals, resistance elements, electro chemical apparatus, chemical containers, and other uses where it is exposed to severe corrosive conditions. Another object is the provision of an alloy having the above characteristics and also sufficiently malleable, ductile, and homogeneous to permit of rolling, drawing, stamping or otherwise working to the desired shape; the provision of an alloy of such homogeneous character as not to be "hot short" or subject to selective corrosion; the provision of an alloy which shall not only conserve the world's supply of platinum but shall be less expensive than platinum; while other objects and advantages will appear as the description proceeds; this application being a division of my two earlier applications Nos.

108,991 and 129,911 filed July 13, 1916 and November 6, 1916, respectively.

The exacting nature of the uses in view immediately exclude from consideration all metals of a readily fusible or oxidizable nature; and alloys of the solid solution type are always preferable to other alloys as being more ductile, malleable, homogeneous and chemically resistant than other types of alloys.

I have discovered that the alloys of gold and palladium, if made of the proper percentage composition, and of the proper degree of purity, (or if certain improper impurities are avoided), will make a complete series of solid solutions of remarkable malleability, ductility and homogeneity; of a hardness fully comparable with that of platinum, a melting point sufficiently high for all practical purposes for which platinum is generally used, an electrical resistivity fully equal to that of platinum, and a chemical resistivity even more pronounced than that of platinum. In view of the fact that a substitute for platinum is the object of this invention platinum itself should not be included to more than a small percentage, although in small quantities it is not injurious. Likewise the metals rhodium, ruthenium and iridium are too rare and costly to be used in large amounts, although they are not deleterious. In fact commercial palladium contains on the average about one half of one per cent. of platinum as an impurity and frequently other noble metals as iridium or rhodium also; it is very rarely free from these substances, especially platinum, and I have known commercial palladium to contain as much as five per cent. of platinum. The cost of refining being greater than the value of the noble metal impurities, I have never taken the precaution of purifying the palladium, and consequently my invention is to be considered as independent of the presence or absence of these substances to a small percentage, whether intentionally or inadvertently present. It is necessary, however, to guard against the presence of base metals, such as iron, cobalt, nickel, copper, lead and other oxidizable substances.

In the drawings accompanying and forming a part of this application, Figure 1 rep-

resents the melting point and hardness curves of the gold-palladium series; Fig. 2 illustrates the melting points and hardness value of pure gold, silver, platinum and palladium upon the same scale; Fig. 3 illustrates the conductivity (both thermal and electrical) of the gold-palladium series; Fig. 4 illustrates the conductivities of pure gold, silver, platinum and palladium upon the same scale; Fig. 5 represents a photomicrograph section showing the segregation of palladium from a chilled solution in gold; Fig. 6 represents a photomicrograph section of the same alloy magnified much more strongly; Fig. 7 represents the condition of the same alloy upon slow cooling; Fig. 8 illustrates a pair of spark points constructed from my improved gold-palladium alloy; and Fig. 9 illustrates a chemical utensil of the said improved material.

The range of temperature through which partial fusion occurs in an alloy of gold and palladium is very small both ascending and descending, and the melting point increases rapidly with the first increment of palladium, so that a decided advantage is afforded by the addition of small proportions of this substance, out of all ratio to its cost. It will also be seen from Fig. 1 that the hardness of the alloy is greater in each case than the hardness of either constituent, being at a maximum substantially at the time that the two metals are present in equal atomic proportions, which is equivalent approximately to palladium 40, gold 60 by weight. A hardness equal to that of platinum is obtained with only twenty per cent. of palladium, while the maximum hardness is about twenty per cent. greater than that of pure platinum.

Reference to Fig. 3 shows that the conductivity of the alloy is much less than the conductivity of either of the component metals, the curve showing a very decided slope at each end, indicating a sudden increase of resistance caused by the admixture of a small amount of the other metal, the conductivity also, as will be expected, reaching a minimum under the condition of equal atomic proportions. In fact an alloy of gold eighty-five per cent. palladium fifteen per cent. (atomic) has the same resistance as pure platinum, while an increase in the palladium content lowers the conductivity only to one third that of platinum; this, coupled with the chemical resistivity of the alloy and its resistance to fusion or oxidation at high temperatures, indicates clearly its value as an electrical resistance wire, for spark points it can be made wide and low to offset this as shown in Fig. 8. In fact the 20 per cent. alloy which is the one most frequently used, is not appreciably inferior to platinum in this regard.

The tendency of the alloy toward segregation upon cooling is very small, but experience proves that if a molten solution of the two substances containing more than about ten atomic per cent. of palladium is suddenly chilled, a slightly segregated condition is secured such as represented in exaggerated fashion in Fig. 5 and in a more highly magnified way in Fig. 6, the center of each metallic crystal being peculiarly rich in palladium and the margins of the crystals grading off to a lower composition. An article so constituted possesses a resistivity to heat, electrical abrasion and chemical action equivalent only to the lowest alloy which it contains; but by cooling the same alloy slowly or by maintaining the alloy for a considerable period at a temperature near but not above its melting point, a re-arrangement of each crystal can be secured and perfect homogeneity obtained as shown in Fig. 7.

For many uses in spark points, electrical contact terminals, philosophical apparatus and dentistry, an alloy of gold and palladium in the proportions of palladium 10 per cent. gold 90 per cent. (atomic) will be sufficient, (equivalent to Pd. 5.6, Au. 94.4 by weight) since such an alloy will have a melting point 100° C. higher than that of pure gold and a hardness substantially midway between that of gold and platinum. Such an alloy, however, is hardly sufficiently resistant physically for use in crucibles and like chemical apparatus, owing to its softness and the danger of accidental melting, although it is of great value in dental foil, its hardness being sufficiently small to permit manipulation, and its melting point being sufficiently high to permit the melting of gold thereon if performed with reasonable care.

For the majority of uses, both electrical and chemical, I recommend an alloy containing approximately gold 80 per cent. (atomic), palladium 20 per cent. (atomic) (equivalent approximately to Au. 88, Pd. 2, by weight), since such an alloy will have a melting point approximately 1250° C. which is sufficiently high to avoid any danger of being melted accidentally under ordinary conditions of use. Such an alloy has a hardness substantially equal to that of platinum, and is of such resistance to chemical, electrical and atmospheric corrosion as to be satisfactory in all cases excepting where the requirements are excessively rigid. For the last named uses I recommend an alloy of gold 60 per cent. (atomic) palladium 40 per cent. (atomic) (equivalent to Au. 73.6 Pd. 26.4, by weight) since such an alloy has a hardness substantially equal to that of platinum alloyed with 10 per cent. of iridium, possesses a melting point of approximately 1350° C.

which is 300° more than that of gold, and will resist practically all the corroding influences which pure platinum will withstand, and many to which pure platinum 5 will succumb.

As heretofore explained I do not limit myself against the use in the above named alloys of small quantities of other noble metals, particularly such as are ordinarily 10 found in association with palladium, so long as the same are used only in small amounts compared with the primary substances herein mentioned. It is necessary, however, that base metals be excluded.

15 Having thus described my invention, what I claim is:—

1. A spark point consisting largely of gold and palladium whose melting point is

above 1150° C. and whose hardness is at least twice that of gold. 20

2. An electric current communicating terminal made of an alloy comprising gold and 20 to 40 atomic per cent. of palladium.

3. Electrical apparatus made of an alloy containing gold and ten to 40 weight per 25 cent. of palladium.

4. Apparatus of the character specified having a working surface consisting of an alloy containing palladium and one or more noble metals surrounding palladium 30 in the periodic table, gold constituting at least 50 At. per cent., and palladium at least 10 At. per cent. of such alloy.

In testimony whereof I hereunto affix my signature.

FRANK A. FAHRENWALD.